

Feb. 28, 1933.

E. P. MARSHALL

1,899,101

METHOD OF FORMING CEMENTITIOUS BODIES AND MATERIAL FOR USE IN SAME

Filed Oct. 4, 1928

2 Sheets-Sheet 1



INVENTOR.

Earl P. Marshall

BY Arthur P. Knigstot and  
Alfred W. Knigstot

ATTORNEYS

Feb. 28, 1933.

E. P. MARSHALL

1,899,101

METHOD OF FORMING CEMENTITIOUS BODIES AND MATERIAL FOR USE IN SAME

Filed Oct. 4, 1928

2 Sheets-Sheet 2

Fig. 6.



Fig. 7.



Fig. 8.



INVENTOR.

Earl P. Marshall

BY Arthur P. Knight and  
Alfred W. Knight

ATTORNEYS

## UNITED STATES PATENT OFFICE

EARL P. MARSHALL, OF LOS ANGELES, CALIFORNIA

## METHOD OF FORMING CEMENTITIOUS BODIES AND MATERIAL FOR USE IN SAME

Application filed October 4, 1928. Serial No. 310,278.

This invention relates to the forming, pouring or casting of cementitious bodies, such as concrete walls, structures, blocks and the like and particularly to a method of forming such bodies in such a manner as to modify the surface thereof and to a material adapted for use in said method. The modification of the surface may consist either in modifying the texture, form, or configuration thereof or in providing any desired coloring thereon, or a combination of both texture and color modification, and it may also include the imparting of water-proof or water-resistant properties to the surface of the concrete.

An important object of the invention is to form cementitious bodies having pleasing surface effects without requiring the subsequent application of surface coatings or coloring thereto or any other treatment after the removal of the forms. This object I accomplish in general by pouring or casting the concrete or other cementitious material of which the body is to be formed, in a form provided with a modifying layer or coating adapted to be transferred to and become bodily incorporated in the surface layer of the concrete body, and to produce the desired surface effect when said body becomes set, so that upon removal of the form the surface of the body will have the desired finished appearance.

A particular object of the invention is to form cementitious bodies in such manner that a pleasing surface of a permanent character is provided thereon, this permanence being due to the fact that the desired effect of color, form, configuration, texture, or resistance to water penetration is produced by surface modifying agents integrally incorporated in the surface layer of such body.

A particular object of the invention is to provide means whereby any one of a wide variety of pleasing surface effects, imitating for example colored building stone, terra cotta, stucco, or block or artificial stone construction of various sorts, may be produced upon the surface of concrete structures or other cementitious bodies, at a minimum

cost, and with a minimum expenditure of time and labor.

Other objects of the invention will be apparent from the description hereinafter.

The accompanying drawings illustrate my invention and referring thereto:

Fig. 1 is a perspective view of a sheet of material adapted for use in lining forms or molds according to my invention.

Fig. 2 is a perspective view of a form for pouring a concrete wall, said form being lined with sheets of material adapted to modify the surface thereof.

Fig. 3 is a face view of a portion of a concrete wall made in a form such as shown in Fig. 2.

Fig. 4 is a face view of one of the walls of a concrete form showing a modified method of placing the sheets of surface modifying material thereon.

Fig. 5 is a face view of a portion of a concrete wall produced by the form shown in Fig. 4.

Fig. 6 is a face view of a portion of one of the walls of a form showing another possible modification in the method of placing the sheets of surface modifying material thereon.

Fig. 7 is a face view of a portion of a concrete wall produced by the form shown in Fig. 6.

Fig. 8 is a view of a portion of a form, or mold, for use in pouring or casting a concrete body, in which the surface modifying coating is applied directly to the interior surface of said form or mold.

According to a preferred embodiment of this invention I employ, for the purpose of lining or covering the interior of forms or molds for use in pouring concrete or other cementitious bodies, material in the form of sheets having a coating of surface-modifying material on the outer face thereof. Each of said sheets, such as indicated at 1 in Fig. 1, may comprise a base of sheet material 2 of suitable thickness to provide the necessary strength without undue weight, for example from  $\frac{1}{16}$  inch, or possibly less in the case of metal sheets, to  $\frac{3}{16}$  inch or more. Said sheets may be of any suitable

size convenient for handling and suitable for the purpose for which they are to be used as hereinafter explained. A convenient size of sheet, for example, may vary from 1 foot 5 to 6 feet in either dimension. It will, of course, be understood that the above figures of thickness and dimensions are given by way of example only and that the invention is not limited in this respect. This sheet 10 material may consist for example of paper, cardboard, boxboard, strawboard, wallboard, or other composition board, or of sheet metal, wood, canvas, or other fabric material, or in general of any sheet material 15 adapted to form a base or backing for application of a coating of surface-modifying material.

The sheet shown in Fig. 1 is provided upon one face with a coating of surface-modifying material 3 applied thereto in such manner 20 as to adhere during shipping or handling of the sheets and during the placing thereof in the forms. Such coating may comprise, for example, a suitable adhesive binding material 25 adapted to form a bond to the sheet 2, and any suitable surface-modifying ingredients incorporated in said binding material. Said binding material may consist, for example, of glue, mucilage, or other adhesive 30 material which is readily soluble in water or adapted to soften upon application of water and the binding material, as well as the surface modifying ingredients, should be adapted to permit substantially normal setting 35 of the concrete in contact therewith so that the binding material and the surface-modifying ingredients carried thereby will actually enter into the surface of the concrete when poured and become an integral part 40 of the surface layer thereof when set.

The surface-modifying ingredients carried by said binding material may include agents adapted to modify either the texture or the color, or both, of the surface of the concrete 45 or other cementitious body. For the purpose of modifying the texture or form, I may use for example, aggregates of various sorts, such as rock, sand, shell, etc., or mixtures thereof, or I may use chemicals which 50 will form gases upon contact of the wet concrete or cementitious material therewith so as to produce a pitted surface.

For modifying the color of the cementitious material I may use colored aggregate 55 such as colored rock, shell or sand, or pigments of suitable color, or any other coloring material, such as dyes, or I may use chemicals adapted to react with one another or with constituents of the cementitious material to produce the desired color effects, all 60 of such color modifying agents being, as above stated, incorporated in the binding material to form the coating 3 on the base 2 of sheet material to be used in lining the 65 forms.

The general method of making the above described sheet material may consist in first applying to the surface of the base material 2, while preferably in the form of relatively large sheets, the binding material such as above mentioned, and then applying thereto the surface modifying agents such as above mentioned as by sprinkling, dusting, blowing or pouring the same thereon, so as to cause such agents to become incorporated therein or to adhere thereto. 75

If desired, however, the surface modifying constituent may first be incorporated or mixed with the binding material and the mixture then applied as a coating on the 80 base material. The expression "incorporated therein", as used herein in this connection, is therefore to be understood as covering either a distribution of the surface-modifying agents throughout all or part of the coating of binding material or simple adherence of such agents to the surface of such coating.

The composite sheets so formed are then dried, after which they may be cut or torn 90 into sheets of any desired size or shape for shipment or use.

The following may be given as a specific example of one form of sheet material according to my invention, for use in lining molds. Sheets of strawboard are coated on one side with a thin coating of common glue, such as sizing glue, which is soluble in water, and aggregate consisting of crushed rock, crushed shell, sand and powdered rock, together with coloring agents consisting of iron sulphate ( $FeSO_4$ ) and vermillion (cinnabar,  $HgS$ ), are sprinkled or dusted over the surface of the wet glue so as to adhere thereto. It will be understood, of course, 100 that any of the other forms of texture modifying or coloring modifying agents above mentioned may be used instead of or in addition to these. Furthermore, the several agents may be applied uniformly over the 110 surface or different agents may be applied on different parts of the surface. Particularly effective results may be obtained, for example, by the selective application of different coloring agents to different portions 115 of the surface so as to produce a mottled effect on the concrete.

The sheets are then subjected to a drying operation so as to cause the glue to harden, after which they may be cut into blocks of 120 suitable size.

In using the sheet material of any of the types above described in the forming of cementitious bodies, the same may be applied in any suitable manner to the interior 125 of forms or molds in which such bodies are to be poured or cast.

In Fig. 2, for example, I have shown a form for pouring a concrete wall. Such form consists as usual of two spaced walls 5 130

each composed of boards laid horizontally and secured to upright supports 6 or to any other suitable supporting means. The sheets 1 are secured to the inner face of one or 5 both of the form walls 5, said sheets being preferably placed with the joints therebetween staggered or offset in successive horizontal rows, as indicated, in the same manner in which bricks or stone blocks are ordinarily laid. The sheets may be secured to the forms in any suitable manner as by means of nails, tacks, clips, or other fastening devices. If both sides of the concrete wall are to be exposed to view, both side 15 walls of the form are preferably lined with the sheet material, while if only one side of the wall is to be exposed or is desired to be finished according to this method, only the corresponding wall of the form needs to 20 be lined in this manner. The walls of the form may be first erected and then lined with the sheet material, or said walls may be assembled in sections and the sheet material applied thereto, and these lined sections then 25 erected in position.

The mixed concrete, consisting of the usual mixture of Portland cement, sand, and aggregate, with water, is then poured between the walls of the form in the usual 30 manner and allowed to harden or set. Upon contact of the wet concrete with the surface modifying coating 3 of the sheet material, such coating is caused to exercise the desired effect upon the surface layer of the 35 concrete, the nature of this effect depending upon the surface-modifying ingredients contained in such coating. The glue or other water soluble binding material will be dissolved or softened by the water in the concrete, and the surface-modifying agents will 40 enter into or adhere to and become incorporated as an integral part of the concrete. Texture modifying agents such as the shell, sand and rock of the above example will be 45 come embedded or will adhere to the surface of the concrete and form a surface of the desired texture, while color modifying agents will penetrate to a greater or less extent into the concrete and impart the desired colors to 50 the surface thereof. If such coloring agents consist of dyes or pigments such as the vermilion in the above example, such materials will simply be transferred to the concrete and form a colored coating or surface 55 thereon.

In any event, the binding material acts as a vehicle for first holding the desired surface-modifying agents in position on the surface of the base material until the concrete 60 is poured, and for then transferring such surface-modifying agents bodily to the wet concrete so as to become integrally incorporated in the surface layer of the concrete body when the same is set. It has heretofore been proposed to apply to the forms,

before pouring the wet cementitious material therein, a coating of cement-destroying material or so-called "medication" adapted to prevent setting or development of a bond in the outer layer of the concrete in contact therewith, so that upon removal of the forms and of the said coating, the outer layer of the cementitious material will either fall off or may be readily removed. This, however, is quite different from my procedure, in which the surface layer of the concrete is permitted to set in normal manner, and in which substantially the entire layer of binding material and surface-modifying material is transferred into the surface 80 layer of the concrete and becomes integrally incorporated in the set concrete body.

If, on the other hand, chemical coloring agents, such as the iron sulphate of the above example are used, these agents will penetrate into the concrete and will there react with constituents of the concrete or with one another to cause precipitation of substances of the desired color. For example, the iron sulphate will react with the alkaline materials in the concrete to probably first form a hydrous ferric oxide which upon drying and exposure to air will be converted to a reddish brown iron oxide, giving a characteristic reddish brown color, which will occur not merely as a thin film or layer upon the surface of the concrete but distributed to a considerable depth therein, so that the color thus imparted will be of a highly permanent 95 nature. It is evident that in this manner any desired color effects may be produced upon the surface of the concrete. A single coloring agent may be provided on the entire surface of all of the sheet material thus giving a plain uniform color effect over the entire surface of the wall, or different coloring agents may be applied to different portions of all of the sheets, producing a mottled effect. A somewhat different effect can also be obtained by the use of only a single 100 coloring agent on each sheet, and placing sheets with different coloring agents in juxtaposition so as to give the effect of blocks of stones of various colors or shades. It is evident that not only the color, but also the texture of different portions of the wall may be varied in a similar manner so as to give 105 pleasing and harmonious effects.

After the concrete has set sufficiently the forms may be removed in the usual manner and the base material of the respective sheets may be stripped from the concrete, leaving a concrete wall with a surface of a texture and color formed as above described. If the sheets are laid in the manner shown in Fig. 2 with their adjacent edges abutting fairly closely and substantially flush with one another, an effect such as shown in Fig. 3 will be produced, the wall having a form or configuration such as to give the appear- 110 115 120 125 130

ance of being formed of blocks or stones of the size and shape of the sheets used for lining the forms, and separated by fine ridges or ledges 8 due to the small cracks 5 or slight departures from a smooth plane of the adjoining edges of adjacent sheets.

As illustrated in Figs. 4 and 5 a somewhat different effect can be secured by spacing the sheets 3 slightly apart in applying 10 the same to a form wall 5 so as to provide grooves or channels 10 therebetween. The concrete wall produced in a form lined in this manner will have the appearance shown in Fig. 5, the effect being that of blocks or 15 stones with raised beads or ridges of pointing material therebetween as indicated at 11.

A different effect can also be secured by applying narrow strips of wood, cardboard or the like as indicated at 12 in Fig. 6 over 20 the joints 13 between adjacent sheets, such strips also serving, if desired, to secure the sheets to the form. Similar strips may also be placed at intervals over the surface of the sheets if desired. As shown in Fig. 7 the 25 wall produced in this manner has the appearance of a wall of blocks or stones, the joints between which are filled with pointing material but are recessed somewhat with respect to the faces of the blocks so as to provide 30 grooves 14 therebetween.

In addition to the above, many varied and artistic effects of form or configuration may be secured by using the sheet material in different ways. For example the material 35 may be torn or cut to form pieces of irregular sizes which may be applied in irregular manner to the forms so as to overlap one another, thus forming an imitation of a rough Spanish texture stucco-finished 40 wall.

If desired, other agents in addition to the texture and color modifying agents above described may also be incorporated in the coating applied to the sheets. Waterproofing agents of various sorts may, for example 45 be applied in this manner. As a specific example, powdered or crushed alum and limestone may be incorporated therein, being applied for example along with the other surface-modifying agents in the example given above, penetrating into the surface 50 layer of the concrete and reacting to form substances adapted to prevent penetration of water therein, due either to water repellent properties thereof or to mechanical closing of the pores of the concrete.

Agents may also be used which are adapted 55 to react with constituents of the concrete or other cementitious mixture to form bubbles of gas which will leave recesses or depressions in the surface of the concrete, giving a pitted effect. Calcium carbide may be used for this purpose, being incorporated with the binding material in the same manner as any of the other surface-modifying

agents above mentioned. Such calcium carbide will react in well known manner with the water of the concrete to form bubbles of acetylene gas. In the specific example given above, powdered or crushed calcium carbide may be sprinkled over the surface of the coating of binding material along with the other surface modifying agents.

As shown in Fig. 8, the surface-modifying coating 8' may be applied directly to 70 the interior of a mold or form instead of applying such coating to sheet material and lining the form therewith. This method of practicing the invention may be used to practical advantage for example, in the casting 80 of blocks or other structural members of concrete or artificial stone composition.

I claim:

1. A material for modifying the surface of cementitious bodies during setting comprising a sheet of base material and a surface modifying coating applied to one face thereof, said coating comprising a binding material adapted to soften upon contact of wet cementitious material therewith, and a water soluble color modifying agent incorporated in said binding material.

2. A material for modifying the surface of cementitious bodies during setting comprising a sheet of base material and a surface modifying coating applied to one face thereof, said coating comprising a binding material adapted to soften upon contact of wet cementitious material therewith, and a water soluble chemical incorporated therein 100 and adapted to react with constituents of wet cementitious material to produce a colored substance.

3. A material for modifying the surface of cementitious bodies during setting, comprising a sheet of base material and a surface modifying coating applied to one face thereof, said coating being free of set inhibiting material so as to permit substantially normal setting of cementitious material in contact therewith and said coating comprising a binding material adapted to soften upon contact of wet cementitious material therewith and water soluble color-modifying material incorporated in said 110 binding material.

4. The method of forming cementitious bodies which comprises providing, on the inner face of a form, a modifying layer comprising a binding material having water soluble material incorporated therein adapted to modify the color of the surface layer of the cementitious material, said binding material being adapted to soften upon contact of water-containing cementitious material therewith, and said modifying layer being adapted to permit substantially normal setting of the cementitious material in contact therewith, supplying water-containing cementitious material to the interior of 130

5 said form in contact with said modifying layer, causing the modifying layer to be bodily transferred from the form to the surface layer of the cementitious material, causing  
10 the cementitious material to harden and the binding material and color-modifying material to become incorporated as an integral part of the hardened surface layer thereof, and then removing the form while  
15 leaving the binding material and color-modifying material permanently incorporated in the surface layer of the said cementitious body.

5. A method of forming cementitious bodies which comprises providing on the inner face of a form, a modifying layer comprising a binding material having incorporated therein water soluble material adapted to modify the color of the surface  
20 layer of cementitious material brought in contact therewith, supplying water-containing cementitious material to the interior of said form in contact with said modifying layer, causing the color-modifying material  
25 to be bodily transferred from the form to the surface layer of the cementitious material, causing the cementitious material to harden, and the color-modifying material to become incorporated as an integral part of  
30 the hardened surface layer thereof, and then removing the form while leaving the color-modifying material permanently incorporated in the surface layer of the said cementitious body.

35 6. The method of forming cementitious bodies which comprises providing, on the inner face of the form, a modifying layer comprising a binding material having incorporated therein material adapted to  
40 chemically react with constituents of wet cementitious material to produce coloring material, supplying water-containing cementitious material to the interior of said form in contact with said modifying layer, causing  
45 the cementitious material to harden and causing coloring material produced as above set forth to become incorporated as an integral part of the hardened surface layer of said cementitious material, and then removing  
50 the form while leaving said coloring material permanently incorporated in the surface layer of said cementitious body.

55 7. The method of modifying the surface of cementitious bodies during setting, which comprises bringing into contact with the surface of a cementitious body during setting thereof a sheet of backing material having  
60 on its inner face a modifying layer comprising a binding material having water soluble material incorporated therein adapted to modify the color of the surface layer of the cementitious material, said binding material being adapted to soften upon contact of water-containing cementitious material therewith, and said modifying layer

being adapted to permit substantially normal setting of the cementitious material in contact therewith, causing the modifying layer to be bodily transferred from said backing material to the surface layer of the  
70 cementitious material, causing the cementitious material to harden and the binding material and color-modifying material to become incorporated as an integral part of the hardened surface layer thereof, and then  
75 removing said sheet of backing material while leaving the binding material and color-modifying material permanently incorporated in the surface layer of said cementitious body.

80 8. The method of modifying the surface of cementitious bodies during setting, which comprises bringing into contact with the surface of a cementitious body during setting thereof a sheet of backing material having on its inner face a modifying layer comprising a binding material having incorporated therein water soluble material adapted to modify the color of the surface layer of cementitious material brought in contact  
85 therewith, causing the color-modifying material to be bodily transferred from the form to the surface layer of the cementitious material, causing the cementitious material to harden and the color-modifying material to become incorporated as an integral part of  
90 the hardened surface layer thereof, and then removing said sheet of backing material while leaving the color-modifying material permanently incorporated in the surface  
95 layer of said cementitious body.

100 9. The method of modifying the surface of cementitious bodies during setting, which comprises bringing into contact with the surface of a cementitious body during setting thereof a sheet of backing material having on its inner face a modifying layer comprising a binding material having incorporated therein material adapted to chemically react with constituents of wet cementitious material to produce coloring material, causing the cementitious material to harden and the coloring material produced as above set forth to become incorporated as an integral part of the hardening surface layer  
105 of said cementitious material, and then removing said sheet of backing material while leaving said coloring material permanently incorporated in the surface layer of said cementitious body.

110 In testimony whereof I have hereunto  
115 subscribed my name this 25th day of September, 1928.

EARL P. MARSHALL.

125

130